

## UNITED STATES PATENT OFFICE

2,411,593

## CORROSION PROTECTION OF METALS

Willis G. Routson, Berkeley, Calif., assignor to  
 Shell Development Company, San Francisco,  
 Calif., a corporation of Delaware

No Drawing. Application August 11, 1943,  
 Serial No. 498,434

11 Claims. (Cl. 252—51)

1

The present invention relates to metals or metal-containing articles of manufacture which are normally subject to corrosion and which have been rendered substantially non-corrodible by treatment with a dispersion of certain nitrogen containing organic compounds in a suitable vehicle. It also relates to compositions having anti-corrosive, and especially rust-protective properties, and more particularly deals with compositions comprising a substantially neutral vehicle such as normally liquid or normally solid hydrocarbons (e.g., fatty oils and natural waxes), alcohols, ethers, water, etc., containing finely dispersed small amounts of such an organic nitrogen compound.

Metallic surfaces, particularly those containing iron, require protection against the hazard of corrosion in the presence of water. To illustrate: Moisture readily attacks finished or semi-finished metal objects unless the metal surface is covered during storage or shipment by a protective coating such as is imparted by a slushing oil; water in Diesel engine fuels often corrodes closely fitted parts such as are found in Diesel engine unit-type injectors; water in turbines corrodes turbine lubricant circulatory systems, particularly the governor mechanisms of steam turbines; water in hydrocarbon oils, such as gasoline, rusts steel storage tanks and drums; water in anti-freeze compositions causes corrosion in automobile radiators, etc. Corrosion not only has a deleterious effect upon the metal surfaces, but also frequently loosens finely divided metal oxides which may act as oxidation catalysts increasing the rate of deterioration of various organic compounds with which they come in contact or they may enter between moving parts of machinery where they act as abrasives.

It is a purpose of this invention to treat metals or articles of manufacture containing metals in a way so that they become resistant to normal corrosion. It is a specific purpose to treat in a simple manner accurately machined metal parts so that they may be handled without developing corrosion, particularly in places where fingerprints have been left. Another purpose is to protect iron or steel equipment exposed to the atmos-

2

phere so that its rusting is prevented or at least retarded. Still another purpose is to protect mechanical equipment from rusting, which equipment stands idle and/or is shipped over long distances. A further object is to provide slushing oils of improved rust-protective properties particularly adapted to withstand the effects of marine environment. Another purpose is to produce lubricating compositions suitable for internal combustion engines which compositions possess improved anti-corrosive, anti-wear and/or other beneficial properties. Still other objects will be apparent from the present description.

This invention is based on the discovery that certain organic nitrogen compounds (as hereinafter described) have valuable and unexpected rust protective and other beneficial properties. These compounds having, say, upward of about 10 carbon atoms and more preferably 12 or more carbon atoms, which are substantially oil-soluble, may advantageously be employed in a lubricating composition or other oily medium. However, the compounds of the invention may be dispersed in either oily or non-oily media although not with the same effectiveness.

The nitrogen compounds of the present invention are characterized by the presence of a nitrile (CN), nitro (NO<sub>2</sub>) or nitroso (NO) group. (Since



may be found in equilibrium with the isomeric form



the latter is considered as included with the nitroso compounds.) These nitrogen-containing radicals are attached to a carbon atom which is not more than three atoms removed from an acidic group. The acidic radical may be COOH, CSOH, COSH, CSSH, SO<sub>3</sub>H, PO<sub>3</sub>H, and the like. Preferably this acidic radical is attached to a carbon atom which is alpha or beta to the carbon atom carrying the nitrile, nitro or nitroso group, since the rust retarding properties are greater

the nearer together these two radicals are. The carboxylic acid radical and the nitrile radical are the preferred radicals of their respective groups.

The present compounds may thus be represented by the formula:



in which  $\text{X}$  is a radical containing an acidic hydrogen atom,  $\text{R}'$  and  $\text{R}''$  (which may be the same or different) are hydrogen atoms or hydrocarbon or substituted hydrocarbon radicals,  $\text{Y}$  is a nitrile, nitro or nitroso radical,  $\text{R}$  is a hydrocarbon or substituted hydrocarbon radical and  $n$  is 0, 1, 2 or 3, but preferably 0 or 1. Preferable values for  $\text{R}'$  and  $\text{R}''$  are hydrogen and/or low molecular weight aliphatic radicals such as methyl, ethyl, propyl, butyl, etc.  $\text{R}$  may also contain an ether type linkage which contains an oxygen, sulfur, selenium or tellurium atom. A preferred group of these latter compounds are those in which this ether linkage is attached to the nitrile, nitro, or nitroso containing carbon atom as represented by the formula



in which  $\text{Z}$  is O, S, Se, or Te.

The several hydrocarbon radicals of the for-

bonyl, amino, hydrosulfide, etc. For maximum stability against deterioration by oxidation, the acid should not contain more than one olefinic double bond per hydrocarbon radical, and more preferably none. Examples of such hydrocarbon

radicals are methyl, ethyl, propyl, isopropyl, normal butyl, isobutyl, secondary butyl, tertiary butyl, normal pentyl, isopentyl, secondary pentyl, hexyl, normal octyl, iso-octyl, normal decyl, isodecyl, dodecyl, tetradecyl, cetyl, stearyl, trimethyl octadecyl, allyl, methallyl, crotyl, methyl vinyl carbonyl, butenyl, pentenyl, hexenyl, propargyl, geranyl, oleyl, phenyl, naphthyl, anthryl, tolyl, xylyl, secondary butyl-naphthyl, dipropyl-naphthyl, benzyl, naphthyl-butyl, phenethyl, vinyl-phenyl, crotonyl-naphthyl, methallyl-phenyl, naphthyl-allyl, 2-phenyl-ethenyl, phenyl vinyl carbonyl, cinnamyl, acetyl, propionyl, caprolyl, stearacyl, benzoyl, ethyl-cyclohexyl, tri-butyl-cyclohexyl, cyclopentenyl, cyclohexenyl, vinyl cyclohexenyl, thionyl, pyrrolyl, pyridyl, furyl, butyl carbothionyl, octyl carbothionyl, decyl carbothionyl, etc.

A preferred group of oil-soluble compounds are those in which the organic radical or radicals have a total of not less than about 8 carbon atoms and more preferably at least 10 or 12 and up to about 60 carbon atoms for good anti-corrosive properties.

These compounds may be produced, for example, by reactions such as the following:



ulae may be aliphatic, alicyclic, aromatic or mixed and may contain substituents which are preferably not too strongly polar, such as halogen, the group



etc., and should preferably be free from highly polar substituents, such as hydroxyl, carboxyl, car-

"Et" in the above formulae stands for ethyl.

Monocarboxylic acids suitable as starting materials for the preparation of the present compounds include fatty acids such as decyl, undecyl, lauric, myristic, palmitic, stearic, arachic, behenic, oleic, phenyl acetic, phenyl propionic, phenyl lauric, phenyl palmitic, phenyl stearic, tolyl stearic, naphthyl acetic, naphthyl stearic, etc., acids. Naphthenic acids, such as are obtained by caustic alkali extraction of relatively

high-boiling straight-run petroleum oils, such as kerosene, gas oil, lubricating oils, etc., may also be used, as well as synthetic naphthenic acids, such as cyclohexyl acetic, cyclohexyl propionic, cyclohexyl stearic acids, corresponding alkyl cyclohexyl, tetrallyl, dicyclohexyl fatty acids, or acids derived from naphthenes obtained by hydrogenation of isophorone, diisophorone and homologues, etc.

Another group of carboxylic acids comprises the group of hydroxy acids such as hydroxy benzoic, hydroxy naphthenic, etc., acids and the alkyl homologues thereof, typical representatives being the alkyl salicylic acids.

The dispersion of the present anti-rusting compounds may be a true or colloidal solution in a suitable vehicle which is capable of flowing under the conditions of use, i. e., is liquid or plastic at the temperature employed. Both true solutions and colloidal dispersion in various vehicles are effective in the matter of corrosion protection. However, true solutions are preferred for two reasons: first, colloidal solutions may, under many circumstances, coagulate, in which case the active protective agent would be eliminated; and second, colloids tend to cause emulsification of oily vehicles with water, emulsification in many instances being very undesirable as in the lubrication of steam turbines.

The treating temperature for metals is preferably about room temperature if the vehicle is normally liquid, although lower or higher temperatures may be employed. The lower temperature limit is usually determined by the solidification temperature of the liquid, and temperatures should be below the boiling temperature of the vehicle and below the decomposition temperatures of both the vehicle and the nitrogen compound.

Metals capable of being thus protected are in particular the ferrous metals, e. g., soft iron, various steels, cast iron, and to a lesser extent copper, brass, bronze, zinc, aluminum, magnesium alloys, various bearing metals as copper-lead, cadmium-nickel, silver-nickel, etc.

Articles containing these metals are too numerous to recite. However, it may be mentioned that the problem of rust prevention is critical, for example, where accurately machined parts are involved such as piston rings, engine cylinders, bearing shafts, plungers of pumps, etc. In other instances, rust prevention may perhaps not be critical, but of vast economic importance as, for example, in the mass production of steel castings which are piled up and often set in the open for months before being finished.

Corrosion may be due not only to atmospheric exposure, but may be caused or accelerated by contact with acidic materials, for example, by touching with the fingers. It may also occur in closed systems, as in internal combustion engines, steam turbines, pipe lines, etc., due to the corrosive influence of various impurities such as water, oxygen, carbon dioxide, salts, inorganic or organic acids, etc.

The treatment, according to this invention, for the prevention of corrosion may consist of a single contact of the metal to be protected with the dispersion containing the nitrogen compound, or may comprise repeated contacts effected at intervals, or may consist of a continuous treatment lasting as long as the use of the particular dispersion or piece of equipment or both. The choice of any particular type of these treatments is usually dictated by circumstances. For example,

if newly machined and finished machine parts are to be rust-proofed, they may be dipped or sprayed with a suitable dispersion, and then stored away. On the other hand, if rust prevention in a steam turbine is desired, it is preferable that the circulating lubricating oil contain the active rust-preventive compound and contact is made as long as this oil is used. Should, after a while, this oil be discarded and be replaced by

another one not containing a rust-preventive, then corrosion protection usually lasts for a long time thereafter, due to the protective film left behind. In cases where this film is mechanically destroyed, as in bearings or gears, etc., running under extreme loads, the protective film must be renewed continuously, otherwise rust protection fails.

The vehicles to which the compounds of this invention may be added for the purpose of producing corrosion-protective compositions may be divided into several groups. In the first place, they may be liquids or plastics, the only requirements as to their physical state being (in addition to their being able to act as carrier for the acids under normal atmospheric conditions) that they be spreadable over metal surfaces. Spreading may be accomplished by immersing, flooding, spraying, brushing, troweling, etc. After being applied, all or part of the vehicle may evaporate, or it may be more or less permanent. In other words, both volatile carriers may be used, or substances which do not materially volatilize under normal atmospheric conditions. As to chemical requirements, the vehicle must be stable under ordinary conditions of storage and use and be inert to the active inhibitors.

Thus the vehicle should preferably be substantially neutral, although it may be weakly acidic or basic, preferably having a dissociation constant not above about  $10^{-8}$ . In vehicles of low dielectric constant, as hydrocarbon oils, which are not conducive to ionization of dissolved electrolytes, relatively small amounts, i. e., about .1% to 5% of various carboxylic acids, such as fatty or naphthenic acids, may be present, and in many instances this may be beneficial.

Both polar and non-polar vehicles may be employed. Among the former are water; alcohols, such as methyl, ethyl, propyl, isopropyl, butyl, amyl, hexyl, cyclohexyl, heptyl, methyl cyclohexyl, octyl, decyl, lauryl, myristyl, cetyl, stearyl, benzyl, etc., alcohols; polyhydric alcohols as ethylene glycol, propylene glycol, butylene glycol, glycerol, methyl glycerol, etc.; phenol and various alkyl phenols; ketones as acetone, methyl ethyl ketone, diethyl ketone, methyl propyl, methyl butyl, dipropyl ketones, cyclohexanone and higher ketones; keto alcohols as benzoin; ethers as diethyl ether, diisopropyl ether, diethylene dioxide, beta-beta' dichlor diethyl ether, diphenyl oxide, chlorinated diphenyl oxide, diethylene glycol, triethylene glycol, ethylene glycol monomethyl ether, corresponding ethyl, propyl, butyl ethers; neutral esters of carboxylic and other acids as ethyl, propyl, butyl, amyl, phenyl, cresyl and higher acetates, propionates, butyrate, lactates, laurates, myristates, palmitates, stearates, oleates, ricinoleates, phthalates, phosphates, phosphites, thiophosphates, carbonates; natural waxes as carnauba wax, candelilla wax, Japan wax, jojoba oil, sperm oil; fats as tallow, lard oil, olive oil, cottonseed oil, perilla oil, linseed oil, tung oil, soya bean oil, flaxseed oil, etc.; weak bases as pyridine, alkyl pyridines, quinolines, pe-troleum bases, etc.

Vehicles of little or no polarity comprise hydrocarbons or halogenated hydrocarbons as liquid butanes, pentanes, hexanes, heptanes, octanes, benzene, toluene, xylenes, cumene, tetraline, indene, hydrindene, alkyl naphthalenes; gasoline distillates, kerosene, gas oil, lubricating oils (which may be soap-thickened to form greases), petrodatum, paraffin wax, albito asphalt, carbon tetrachloride, ethylene dichloride, propyl chloride, butyl chloride, chlor-benzol, chlorinated kerosene, 10 chlorinated paraffin wax, etc.

The amounts of the present compounds which must be incorporated in the above vehicles to produce corrosion-protective compositions vary considerably with the type of vehicle used. As a general rule, the presence of resinous materials, particularly those of a colloidal nature, calls for relatively larger amounts of inhibitors. Resinous materials which interfere with the activity of the inhibitors comprise asphaltenes, petroleum resins, 20 various other natural resins, as rosin, resins formed by polymerization of drying fatty oils, phenol-formaldehyde resins, glyptal type resins formed by esterification of polyhydric alcohols with polycarboxylic acids, etc.

In the absence of such resinous materials, amounts required of the nitrogen compounds vary from about 0.001% up to about 0.1%, although larger amounts may be used. However, where the rust retarding compounds are in colloidal dispersion, rather than in true solution, a concentration in excess of about 0.1% may result in relatively quick loss of part of the inhibitor by precipitation and settling.

In the presence of resins and other colloids, amounts in excess of 0.1% and up to say 5% may be required. Inasmuch as resins may act as protective colloids, compositions containing these larger amounts of colloidally dispersed inhibitors, together with resin, may be quite resistant to precipitation and settling.

Since resinous and gummy substances in the vehicles do call for greater amounts of inhibitors, it is usually desirable to refine normally liquid vehicles thoroughly and free them from gummy substances, thereby imparting to them maximum inhibitor susceptibility. This is of particular importance, for example, in lubricating oils, specifically steam turbine oils, which are advantageously highly refined before the inhibitor is introduced. Suitable refining treatments include, for example, extraction with selective solvents for aromatic hydrocarbons such as liquid sulfur dioxide, phenol, furfural, nitrobenzene, aniline, beta-beta'-dichloro-diethyl ether, antimony trichloride, etc.; treatment with  $AlCl_3$ , sulfuric acid, clay, etc. If the treatments produce a sludge, special care must be taken to remove it very thoroughly and completely.

It has also been found advantageous to incorporate together with the nitrogen compound in an appropriate medium, particularly in a lubricating oil or other nongaseous hydrocarbon (e. g., gasoline, Diesel fuel, kerosene, gas oil, petroleum, plastics, petrodatum, etc.) small amounts of certain oil-soluble dicarboxylic acids or hydroxy aromatic carboxylic acids possessing corrosion protective properties. Acids possessing this property are those having at least 12, and preferably 20 or more carbon atoms, and it is desirable that their active radicals, i. e., the several carboxylic radicals, or carboxylic and hydroxyl radicals, as the case may be, be as close to each other as possible and be separated from each other by not more than 4, and preferably by not more than 2,

intervening atoms. Stability of the acids under conditions to which the compositions are exposed is an added requirement.

Among the dicarboxylic acids which are particularly useful for preventing corrosion are various alkylated aliphatic dicarboxylic acids such as alkylated succinic, glutaric, adipic, etc. acids. If desired, these acids may contain various substitution radicals as hydroxyl, ether, amino, nitro, hydrosulfide, sulfide, halide, etc., radicals, the most important limiting factor being the necessary stability. In general, it is preferred to use a saturated aliphatic dicarboxylic acid having the carboxyl radicals as close to each other as possible as is consistent with the requirement for stability. Particularly effective are alkyl succinic acids having at least 16, and preferably 20 to 40 carbon atoms.

Of the hydroxy carboxylic acids, hydroxy aromatic carboxylic acids in which the hydroxy radical is directly attached to the aromatic nucleus are most useful; for example, various alkyl phenol or naphthol carboxylic acids wherein the carboxylic acid radical is attached to the nucleus directly or through a carbon linkage, e. g., alkyl salicylic acids, preferably those whose alkyl radicals contain 12 or more carbon atoms.

The addition of these auxiliary acids to hydrocarbon oils containing the primary anti-corrosives is of greatest importance when dealing with well-refined hydrocarbon compositions. Conventional refining methods, such as acid and alkali treatment, solvent extraction, hydrogenation, etc., remove naphthenic and other monocarboxylic acids which may naturally be contained in the hydrocarbons in small amounts and which may enhance the action of the anti-corrosives. However, even if small amounts of naphthenic and similar acids are naturally present, in general the addition of further amounts of the auxiliary acids of the type described is beneficial. Without wishing to be committed to a particular theory of why this combination of nitrogen compound and dicarboxylic acid produces such an effective anti-rusting combination, it seems that the nitrogen compound more rapidly forms a protective film than the dicarboxylic acid so that the nitrogen containing compound yields better initial (or quicker) protection while the dicarboxylic acid produces enhanced ultimate protection.

The nitrogen compound, in addition to affording rust protection itself, also promotes the formation of a protective film of the dicarboxylic acid on a metallic surface. This combination of nitrogen compound and dicarboxylic acid is particularly important in connection with the rust inhibiting of highly refined lubricating compositions such as turbine oil since the refining treatment may render the nitrogen compound only sparingly soluble in the finished oil. Thus a refined Mid-Continent 400 vis. at 100° F. turbine raffinate may only dissolve about 0.015% of alpha stearic acid while it will dissolve about 5% alkyl succinic acid obtained by condensation of maleic anhydride with higher molecular weight olefins (Ex  $C_{12}$ - $C_{30}$ ) and subsequent hydrolysis to the acid.

In general, amounts of these auxiliary dicarboxylic acids between about 0.001% and 0.1% may be used in petroleum distillate oils; in bright stocks up to about 1% is indicated, while in plastic compositions higher amounts, even up to 5-10%, may be useful.

The invention may be further illustrated by reference to the following modified Kuebler or

Westinghouse corrosion tests. Steel strips (3" x 1/2" x 1/8") were completely immersed in 460 ml. samples of oil which were continuously agitated with electric motor-driven glass stirrers. Thirty minutes after starting, 10% volume of synthetic sea water was added to each sample. The tests were continued for 48 hours at a controlled temperature of 75° C. and the amount of rusting on the strips then noted. (The synthetic sea water was made up from the following formula: in 1000 ml. water—11.0 g.  $MgCl_2 \cdot 6H_2O$ ; 4.0 g.  $Na_2SO_4$  (anhydrous); 1.2 g.  $CaCl_2$  (anhydrous); 25.0 g.  $NaCl$ .)

Results were as follows:

| Additive                         | Concentration, percent, by weight | Base oil                                                                                      | Result                                                         |
|----------------------------------|-----------------------------------|-----------------------------------------------------------------------------------------------|----------------------------------------------------------------|
| $\alpha$ Cyano stearic acid      | 0.015                             | Mid-Continent 400 vis. at 100° F. turbine raffinate.                                          | Perfect.                                                       |
| Do                               | 0.010                             | do                                                                                            | Do.                                                            |
| Alkyl succinic acid 1            | 0.022                             | do                                                                                            | About 10% rusted in first 4 hours of test (test then stopped). |
| Alkyl succinic acid 1 plus       | 0.01                              | do                                                                                            | Perfect.                                                       |
| $\alpha$ Cyano stearic acid      | 0.0075                            | do                                                                                            | Do.                                                            |
| Do                               | 0.015                             | California turbine raffinate containing 0.25% by weight of tertiary butyl phenol (inhibitor). | About 15% rusted after 48 hours.                               |
| Do                               | 0.010                             | do                                                                                            | Perfect.                                                       |
| $\alpha$ Cyano stearic acid plus | 0.0075                            | do                                                                                            |                                                                |
| Alkyl succinic acid 1            | 0.01                              | do                                                                                            |                                                                |

<sup>1</sup> Approximate molecular weight 600

When the anti-corrosive agents of the present invention are employed in a lubricating oil for internal combustion engines, other additives may also be present, such as blooming agents, pour-point depressants or viscosity improvers, anti-oxidants, extreme pressure agents, detergents, anti-foaming agents, etc. Thus, oil-soluble detergents may include the oil-soluble salts of various bases with detergent forming acids. Such bases include metal as well as organic bases. Metal bases include those of the alkali metals, Cu, Mg, Ca, Sr, Ba, Zn, Cd, Al, Sn, Pb, Cr, Mn, Fe, Ni, Co, etc. Organic bases include various nitrogen bases as primary, secondary, tertiary and quaternary amines.

Examples of detergent forming acids are the various fatty acids of say, 10 to 30 carbon atoms, wool fat acids, paraffin wax acids (produced by oxidation of paraffin wax), chlorinated fatty acids, rosin acids, aromatic carboxylic acids including aromatic fatty acids, aromatic hydroxy fatty acids, paraffin wax benzoic acids, various alkyl salicylic acids, phthalic acid mono ester, aromatic keto acids, aromatic ether acids; diphenols as di-(alkylphenol) sulfides and disulfides, methylene bis alkylphenols; sulfonic acids such as may be produced by treatment of alkyl aromatic hydrocarbons or high boiling petroleum oils with sulfuric acid; sulfuric acid mono esters; phosphoric, arsonic and antimony acid mono and di esters, including the corresponding thio phosphoric, arsonic and antimony acids; phosphonic and arsonic acids; etc.

Other detergents are the alkali earth phosphate di esters, including the thiophosphate di esters; the alkali earth diphenolates, specifically the calcium and barium salts of diphenol mono and poly sulfides.

Non-metallic detergents include compounds such as the phosphatides (e. g., lecithin), certain fatty oils as rapeseed oil, voltolized fatty or mineral oils, etc.

Anti-oxidants comprise several types, for example alkyl phenols such as 2,4,6-trimethyl

phenol, pentamethyl phenol, 2,4-dimethyl-6-tertiary butyl phenol, 2,4-dimethyl-6-octyl phenol, 2,6-ditertiary butyl-4-methyl phenol, 2,4,6-tritertiary butyl phenol, etc.; amino phenols as benzyl amino phenols; amines such as dibutyl phnylene diamine, diphenyl amine, phenyl alpha naphthyl amine, phenyl beta naphthyl amine, dinaphthyl amines; various sulfurized compounds, as sulfurized sperm oil, sulfurized jojoba oil, sulfurized resins or olefin polymers, paraffin wax polysulfides, sulfurized tall oil, sulfurized terpene hydrocarbons, methylene bis phenyl sulfides, etc.

Other corrosion inhibitors may also be present.

such as alkali metal and alkali earth salts of sulfonic acids and fatty acids, etc.

I claim as my invention:

1. A corrosion-preventive composition comprising a predominant amount of a hydrocarbon fraction containing finely dispersed a corrosion retardant amount of an organic monobasic acid of between about 10 and about 60 carbon atoms and containing a radical selected from the group consisting of nitrile, nitro, and nitroso radicals which is not more than four carbon atoms removed from the acid radical.

2. The composition of claim 1 wherein said corrosion retarding acid is an alpha cyano carboxylic acid containing a minimum of 12 carbon atoms.

3. The composition of claim 1 wherein said vehicle is normally liquid.

4. A lubricating composition comprising a predominant amount of a refined mineral oil and a beneficiating amount of an oil-miscible compound having between about 10 and about 60 carbon atoms of the formula



wherein R' and R'' are selected from the group comprising hydrogen atoms, hydrocarbon and substituted hydrocarbon radicals, R is an organic radical, X is a radical containing an acidic hydrogen atom, Y represents a radical selected from the group consisting of a nitrile, nitro and nitroso radical and n represents a number selected from the group consisting of 0, 1, 2 and 3.

5. The composition of claim 4 in which said compound is an alpha cyano carboxylic acid.

6. The composition of claim 4 in which said mineral oil is a turbine oil.

7. The composition of claim 4 in which said compound has a minimum of 12 carbon atoms and is present in the amount of about 0.001% to about 0.1%.

8. The composition of claim 4 which also contains a small amount of a corrosion inhibiting

11

dicarboxylic acid containing a minimum of 16 carbon atoms.

9. An improved turbine oil comprising a refined mineral lubricating oil in which has been incorporated about 0.001-0.1% of an oil miscible alpha cyano carboxylic acid having between about 10 and about 60 carbon atoms and about 0.001-0.1% of an oil soluble alkyl succinic acid possessing a minimum of 16 carbon atoms.

10. A corrosion-preventive composition comprising a predominant amount of a substantially neutral vehicle containing finely dispersed therein a corrosion retarding amount of an organic monobasic acid having between about 10 and about 60 carbon atoms and containing a radical selected from the group consisting of nitrile, nitro and nitroso radicals which is not more than 4

5

10

15

12

carbon atoms removed from the acid radical, and a small amount of a dicarboxylic acid containing at least 16 carbon atoms.

11. A corrosion-preventive composition comprising a predominant amount of a hydrocarbon fraction containing finely dispersed therein a corrosion retarding amount of an organic monobasic acid having between about 10 and about 60 carbon atoms and containing a radical selected from the group consisting of nitrile, nitroso and nitro radicals which is not more than 4 carbon atoms removed from the acid radical, and from about 0.001% to about 0.1% of an alkyl succinic acid having a minimum of about 16 carbon atoms.

WILLIS G. ROUTSON.